

## UNITED STATES PATENT OFFICE

HENRY AUGUST MUELLER, OF STOCKHOLM, SWEDEN; ASSIGNOR TO AKTIEBOLAGET  
FERRICONCENTRAT, OF STOCKHOLM, SWEDEN

METHOD OF ENRICHING IRON ORE, BLAST FURNACE FLUE DUST, BURNT PYRITE,  
PURPLE ORE AND THE LIKE

No Drawing. Application filed August 22, 1927, Serial No. 214,778, and in Sweden October 28, 1926.

Certain iron-ores are, as well known, in their natural state only feebly paramagnetic so that they either not at all or only by use of high intensity magnetic separators can be enriched in the magnetic way. To this class belong the iron ores of the types  $Fe_2O_3$  (brown and red hematites, iron-glances etc.),  $FeO_2CO$  (spathic ores etc.) and hydrate ores. This is also true of blast furnace flue dust, 10 burnt pyrites and purple-ore, which essentially consist of ferric oxide ( $Fe_2O_3$ ). As the magnetic separation of such ores by means of high intensity magnetic separators is very expensive and often gives a bad result, magnetic methods have heretofore not been generally used for their enrichment, or they have been transferred by partial reduction with carbon (spathic ores being first heated and oxidized to  $Fe_2O_3$  and then partially reduced) more or less completely to ferroso-ferric oxide ( $Fe_3O_4$ ) so as to render them sufficiently paramagnetic to be separated in low intensity magnetic separators. It has been proved by experience that in the latter case at least half of the ore must be transferred into ferroso-ferric oxide to obtain a satisfactory result. Such a reduction process generally requires a rather large quantity of carbon (about 3-5% by weight of the ore) and a rather long time of treatment and high temperature, and can, therefore, only be used in exceptional cases.

The object of this invention is to render an enrichment of iron-ores and ferric oxide materials of the above-mentioned kind possible within low intensity magnetic separators, without any preceding reduction being necessary. The invention is based on the discovery that the cited ferric oxide materials can be transferred by heating into a highly paramagnetic ferric oxide.

It is sufficient for obtaining this effect to heat the ferric oxide or the ferric oxide ore to a comparatively moderate temperate (about  $600^{\circ} C.$ ) and during a short time (about  $1/4$  to  $1/2$  hour). The heating is, preferably, effected in an indirect way. It has been found that the best results are obtained, if the heating of the ferric oxide takes place in presence of a small amount of carbonaceous

material in solid, liquid or gaseous state (for instance  $1/4$ - $1/2$ % by weight of coal powder). The cooling of the heated material can also be made in the air without any change of the high paramagnetism obtained taking place. 55 That the result achieved by the present method is not due to any chemical change is evident both from the chemical analysis which gives an essentially unchanged chemical composition and from spectro-graphic investigations, which show that the treated material has still the rhombic crystal form of the ferric oxide. A minette ore treated according to the invention was found at the analysis to contain 73.10%  $Fe_2O_3$  and only 2.06%  $FeO$ , 60 another contained 76.06%  $Fe_2O_3$  and 1.54%  $FeO$ . An öölit-ore, which was treated in the above manner was found at the analysis to contain 74.4%  $Fe_2O_3$  and only traces of  $FeO$ . It was found at the microscopic investigation 70 that the iron mineral had in this last case been re-crystallized in such a way that iron-glance had been produced. This sample was very strongly paramagnetic and had even a remnant magnetism after magnetic separation. 75

When spathic iron-ore is treated according to this method, it is first to be calcined in presence of air, so that ferric oxide ( $Fe_2O_3$ ) is produced. This calcination can be effected 80 either separately or in the same operation, which brings forth the paramagnetism of the ferric oxide. In the latter case it should be observed that the last part of the heating process for transferring the oxide produced 85 to paramagnetic ferric oxide should, preferably, be performed without admission of air.

Hydrate ores are when heated transferred directly to ferric oxide while water is driven off and, therefore, their transferring to paramagnetic ferric oxide can be made in a single operation. 90

Blast furnace flue dust contains generally such a large amount of carbon that it is sufficient for reducing all ferric oxide therein to 95 ferrous oxide. When treating such material according to this invention such a short heating time and such a low temperature are to be used, that substantially no reduction takes place and, therefore, if the heating is made 100

without admission of air the carbon is consumed in but a little degree, viz to bind the oxygen of the air present between the particles of the material treated. By admitting air in a regulated amount part of the carbon can be combusted to generate some or all of the heat required for the heating. Another way generally more advantageous of utilizing the carbon content of the blast furnace flue dust is to use the flue dust as an addition to other ores not containing carbon in such quantity that the mixture contains about  $\frac{1}{4}$  to  $\frac{1}{2}\%$  by weight of carbon. If the carbonaceous blast furnace flue dust is added in a larger amount part of the carbon can also in this case be combusted by admission of air to generate the heat necessary for the process. When non-carbonaceous ores are treated without addition of carbonaceous blast furnace flue dust part of the fuel necessary for the heating is mixed with the ore and combusted by a regulated admission of air.

For the heating any suitable furnace construction can be used. As the temperature required for the treatment is rather low the furnace can be built entirely or partly of iron.

It is generally advantageous to cool the heated ore in air in order to transfer the ferroso-ferric oxide which may be formed in small quantities, to ferric oxide. If this cooling is carried out according to the counter-current principle and not too rapidly the mineral often is rendered more strongly magnetic than by cooling without admission of air or in water. The air used for cooling the ore and thus preheated can be used for the combustion of the fuel which is required for the heating of the ore or to preheat the ore to be treated whereby a considerable saving of fuel can be obtained.

After transferring of the material to paramagnetic ferric oxide the magnetic separation is effected in common low intensity magnetic separators. In the practical use of the invention ferric oxide materials have been obtained with a stronger paramagnetism than that of ferroso-ferric oxide and the output in separating the material in a low intensity magnetic separator has reached a value of 95 to 97.5%.

What I claim is:

1. Method of treating oxide iron ores, blast furnace flue dust, burnt pyrites, purple ore and the like which in their natural state are only weakly paramagnetic, which comprises heating the material to about  $600^{\circ}$  C. substantially in absence of free oxygen while maintaining the oxidation of the iron mineral substantially at the stage of  $Fe_2O_3$ , and then separating it in a low intensity magnetic separator.

2. Method of treating oxide iron ores of the carbonate type, which comprises transferring the iron mineral of the ore substantially into ferric oxide ( $Fe_2O_3$ ) by heating in pres-

ence of air, then continuing the heating at a temperature of about  $600^{\circ}$  C. substantially in the absence of free oxygen while maintaining the oxidation of the iron mineral substantially at the stage of  $Fe_2O_3$ , and finally separating the material in a low intensity magnetic separator.

3. Method of treating oxide iron ores, blast furnace flue dust, burnt pyrites, purple ore and the like which in their natural state are only weakly paramagnetic, which comprises heating the material to about  $600^{\circ}$  C., in presence of carbonaceous material in quantity sufficient to bind the free oxygen between the ore particles but insufficient to essentially alter the oxidation stage of the iron mineral, and then separating the material in a low intensity magnetic separator.

4. Method of treating oxide iron ores and the like, which in their natural state are only weakly paramagnetic, which comprises mixing non-carbonaceous oxide iron ore with carbonaceous blast furnace flue dust in such quantity that the carbon content of the mixture is sufficient to bind the free oxygen present between the ore particles but insufficient essentially to alter the oxidation stage of the ore, heating the mixture to about  $600^{\circ}$  C. while excluding the atmospheric air, and finally separating the material in a low intensity magnetic separator.

In testimony whereof I have signed my name.

HENRY AUGUST MUELLER.

100

105

110

115

120

125

130